

June 21, 1938.

J. F. POLLARD

2,121,668

METHOD OF TREATING LEATHER BOARD

Filed April 15, 1936

*Fig. 1*



*Fig. 2*



*Fig. 3*



INVENTOR

By *Joseph F. Pollard*  
*Samuel G. Oden*  
ATTORNEY

## UNITED STATES PATENT OFFICE

2,121,668

## METHOD OF TREATING LEATHER BOARD

Joseph F. Pollard, Newburyport, Mass., assignor,  
by mesne assignments, to The International  
Leather Company, Boston, Mass., a corpora-  
tion of Maine

Application April 15, 1936, Serial No. 74,495

9 Claims. (Cl. 8—107)

This invention relates to a vari-colored leather board product and method of producing the same and has particularly to do with providing an improved and novel process employed in the manufacture of heels for shoes. Heretofore it has been proposed to make a vari-colored or striped product by staining one or both flat faces of leather board with a coloring liquid, such as paint or lacquer, which penetrates but partially the thickness of the leather board, as disclosed in Patent No. 1,844,366 to Walter P. Rankin. The present invention may be employed with or without coloring material to produce a vari-colored or vari-shaded striped board, that is, it may be employed either in conjunction with the process generally and broadly disclosed in said Rankin patent, or without the employment of any added coloring material to produce the vari-colored or vari-shaded product of this invention.

Also, it has heretofore been proposed to bleach or treat the flat side surfaces of leather board with aqueous solutions of acids which are not only offensive, but actually injurious to the workmen engaged in the treatment therewith of leather board for heelng purposes. Moreover, such acids tend to injuriously affect the quality of the leather board so treated, particularly to render it more brittle.

The present invention provides a superior product and process and not only obviates the necessity and disadvantages of using such acids, but also may be practiced more cheaply and, moreover, produce a materially better product more closely approaching the characteristics of genuine leather, particularly in that it is more flexible, firmer, tougher and more resistant to abrasion than leather board which has been subjected to treatment, particularly acid treatment, as heretofore proposed and practiced.

In the practice of the process of this invention there preferably is provided a leather board made from colored stock so that the resultant leather board made in the paper making process is colored through and through to substantially the same color, for example, to a reddish or an orange color as distinguished from the ordinary gray board, though the latter may be employed and treated in substantially the same manner. In accordance with the preferred practice of this invention, in order to change the color and/or shade of the leather board, said board is then subjected to treatment with an aqueous solution of sodium bi-fluoride by dipping or painting the board with the said solution, the concentration of which is preferably that obtained by mixing

four to six ounces of powdered sodium bi-fluoride in a gallon of water. The solution thus obtained is not only substantially odorless and inoffensive, but also entirely harmless to workers coming in contact with the same. Moreover, the cost of the solution is substantially less than is the case with treatments in use heretofore. If desired, though it is not necessary, color, for example yellow and/or orange aniline acid dye, may be added to the sodium bi-fluoride solution in the amount of  $\frac{1}{8}$  to  $\frac{1}{2}$  ounce of dye per gallon, and it is found that the sodium bi-fluoride assists in the penetration and/or setting of the dye. A typical example of the solution is as follows:

|                                |        |               |    |
|--------------------------------|--------|---------------|----|
| Sodium bi-fluoride             | ounces | 4 to 6        | 15 |
| Azo yellow dye                 | do     | $\frac{1}{4}$ |    |
| Orange Y, Colour Index No. 151 | do     | $\frac{1}{8}$ |    |
| Water                          | gallon | 1             |    |

The solution thus made up is then preferably heated to a temperature of 110°—125° F. and is then ready for use and may be applied to the board by dipping or painting, as desired, dependent somewhat upon whether one or both sides of the board are to be treated. Ordinarily the depth of penetration desired is of the order of  $\frac{1}{8}$  to  $\frac{1}{4}$  of an inch and, it is found in practice, for example, that leather board three sixteenths of an inch thick may be suitably treated for a period of one and one-half to two and one-half minutes in the solution as just described and, upon drying, thus assume the desirable and superior physical characteristics before referred to, and provide a lighter colored or shaded portion wherever treated. From such sheet material which presents an edge-stripe at its cut section there may be cut heel lifts having an outside surface or surfaces thereof of a color or shade contrasting with that of the darker center portion of the board. If desired to lighten the color and/or shade to a desired depth of the board throughout its thickness, the penetration may be carried entirely through the board and may be very quickly accomplished, particularly when no dye is employed in the solution.

The accompanying drawing illustrates heel lifts as one example of a product of the process hereinbefore described. In said drawing, Figure 1 is a perspective view of a portion of a sheet of leather board before treatment, Fig. 2 is a perspective view of a heel lift cut from board that has been treated throughout its thickness, and Fig. 3 is a perspective view of a heel lift cut from board that has been treated in a manner to present three transverse stripes on its cut section.

The illustration of the untreated board 10 (Fig. 1) shows a dark edge face 12, as would appear at a cut section of untreated board, for comparison with the much lighter color or shade of the edge face 14 of the lift 15 (Fig. 2) which has been cut from board left in the solution long enough to effect a through and through penetration. The lift 20 (Fig. 3) is cut from board previously dipped in the solution for a briefer period of time and presents at its edge face a central stripe 21 and two outer or marginal stripes 22 and 23. The two outer stripes, representing the treated board stock, are here shown as of a lighter color or shade than the central stripe which represents the untreated board stock. Obviously a heel lift or other product having a two-stripe edge face may be produced by painting only one side face of the board, the penetration of the solution partly through the board from that face only leaving the remainder of its thickness of the color of the fibres as originally processed to make the leather board.

In lieu of the sodium bi-fluoride herein referred to, there may be employed potassium bi-fluoride, ammonium bi-fluoride, or a combination of said bi-fluorides, namely the alkali metal acid salts of hydrofluoric acid and the ammonium acid salt of hydrofluoric acid.

Having described my invention what I wish to claim and secure by Letters Patent is:—

1. The method of making a striped leather board product which consists in first providing a leather board of uniform color throughout, then treating the said leather board through only a portion of its thickness with an aqueous solution comprising at least one acid salt selected from the group consisting of the alkali metal acid salts of hydrofluoric acid and the ammonium acid salt of hydrofluoric acid, and finally drying the same.

2. The method of making a striped leather board product which consists in first providing a leather board of uniform color throughout, then treating the said leather board through only a portion of its thickness with an aqueous solution comprising a coloring material and at least one acid salt selected from the group consisting of the alkali metal acid salts of hydrofluoric acid and the ammonium acid salt of hydrofluoric acid, and finally drying the same.

3. The method of making a leather board product which consists in first providing a leather board of uniform color throughout, then treat-

ing the said leather board to a substantial depth with an aqueous solution comprising at least one acid salt selected from the group consisting of the alkali metal acid salts of hydrofluoric acid and the ammonium acid salt of hydrofluoric acid, and finally drying the same.

4. The method of making a striped leather board product which consists in first providing a colored leather board of uniform color throughout and then treating the said leather board through only a portion of its thickness with an aqueous solution of sodium bi-fluoride, and finally drying the same.

5. The method of making a striped leather board product which consists in first providing a leather board of uniform color throughout and then treating the said leather board through only a portion of its thickness with an aqueous solution comprising aniline dye and at least one acid salt selected from the group consisting of the alkali metal acid salts of hydrofluoric acid and the ammonium acid salt of hydrofluoric acid, and finally drying the same.

6. The method of making a striped leather board product which consists in first providing a leather board, then treating said leather board through only a portion of its thickness with an aqueous solution of sodium bi-fluoride, and then drying the same.

7. The method of making a leather board product which consists in first providing a leather board, then treating said leather board throughout its thickness with an aqueous solution of sodium bi-fluoride, and then drying the same.

8. The method of making a leather board product which consists in first providing a leather board, then treating said leather board throughout its thickness with an aqueous solution comprising at least one acid salt selected from the group consisting of sodium bi-fluoride, potassium bi-fluoride and ammonium bi-fluoride, and then drying the same.

9. The method of making a leather board product which consists in first providing a leather board, then treating said leather board through only a portion of its thickness with an aqueous solution comprising at least one acid salt selected from the group consisting of sodium bi-fluoride, potassium bi-fluoride and ammonium bi-fluoride, and then drying the same.

JOSEPH F. POLLARD.

CERTIFICATE OF CORRECTION.

Patent No. 2,121,668.

June 21, 1938.

JOSEPH F. POLLARD.

It is hereby certified that error appears in the printed specification of the above numbered patent requiring correction as follows: Page 1, second column, line 41, strike out the words "to a desired depth" and insert the same after "shade" in line 38; and that the said Letters Patent should be read with this correction therein that the same may conform to the record of the case in the Patent Office.

Signed and sealed this 26th day of July, A. D. 1938.

(Seal)

Henry Van Arsdale,  
Acting Commissioner of Patents.